

Jan. 15, 1935.

S. McMULLAN ET AL

1,987,628

METHOD OF MANUFACTURING NONFERROUS ALLOY SHEETS AND STRIPS

Filed Jan. 13, 1933



INVENTORS  
S. MC MULLAN  
E. S. STRANG

BY  
H. A. Whitehorn

ATTORNEY

## UNITED STATES PATENT OFFICE

1,987,628

## METHOD OF MANUFACTURING NONFERROUS ALLOY SHEETS AND STRIPS

Samuel McMullan, Downers Grove, and Elmore Steele Strang, Oak Park, Ill., assignors to Western Electric Company, Incorporated, New York, N. Y., a corporation of New York

Application January 13, 1933, Serial No. 651,504

15 Claims. (Cl. 29—18)

This invention relates to a method of forming articles, and more particularly to a method of forming thin sheets and tape of non-ferrous metal.

5 An object of the invention is to provide a method for forming articles, such as sheets and tape, of non-ferrous metal with a minimum of labor and expense.

One embodiment of the invention contemplates 10 a method of forming sheets or strips of certain non-ferrous alloys which comprises casting the alloy into a billet substantially free of impurities and containing not more than 0.1 per cent of lead, and hot rolling the billet into a sheet or 15 strip while maintaining it within a predetermined temperature range above the temperature at which the particular alloy becomes brittle while being worked, hereinafter referred to as the "critical" temperature. After the sheet has been 20 allowed to cool below the annealing temperature, it may be cold rolled to the desired gauge by successive heavy reductions without intermediate annealing operations. If a soft sheet is desired it is annealed after the completion of the 25 final cold rolling operation, when the metal has been reduced to the desired thickness. Where a definite degree of hardness is required, the sheet is cold rolled down to a thickness slightly above the desired gauge, is then annealed, and is finally 30 brought down to the desired gauge. This produces a degree of hardness which approximately corresponds to the amount of reduction after the annealing step.

The invention will be more fully understood 35 from the following description, taken in conjunction with the appended drawing, in which the single figure diagrammatically illustrates the various steps of the process.

Referring more particularly to the drawing, 40 the reference numeral 1 represents a furnace wherein the billets of non-ferrous metal are first heated to a hot rolling temperature, the precise temperature depending upon the composition of the particular alloy being treated, the speed of 45 handling and rolling, and other factors. A heated billet 2 is then removed from the furnace and passed through the hot rolls 3—4, which may be arranged in tandem or otherwise and which reduce it by heavy drafts or passes to a sheet of 50 about 5 to 10 per cent of the original thickness of the billet without lowering its temperature below the "critical" temperature of the particular metal being treated. The sheet is then allowed to cool in air, which anneals the metal without 55 the necessity for a special heating and annealing

step, and is then immersed in a pickling bath 7. After pickling, the sheet is passed through cold rolls 9, 10 and 11, which may be of the cluster or other backed-up type, wherein the metal is reduced by a few heavy passes substantially to its final gauge, which may be about 10% of its thickness before cold rolling. It has been found that such radical reductions may be made in the cold rolls without the necessity for any intermediate annealing such as has been customary in the past.

5 In case it is desired to impart to the finished article a definite degree of hardness, the sheet is brought, by rolls 11, to a thickness or gauge only slightly greater than that desired, is then annealed in an annealing oven 12, and thereafter passed through cold rolls 14, which may be of the backed-up type, to bring the sheet to the desired gauge. The final rolling operation on rolls 14 produces in the metal a degree of hardness which 10 corresponds to the amount of reduction made thereby; that is, the greater the reduction the harder the finished product.

15 When employing the method of the present invention for forming sheets of copper-zinc alloys containing 63 to 68 per cent of copper, it is essential that the alloys be substantially free of impurities. It has been found that the presence of more than 0.1 per cent of lead will usually 20 render it impossible to work these alloys in the manner described above. This is true, also, for copper-nickel-zinc alloys containing 53.5 to 73.5 per cent of copper and 16.5 to 19.5 per cent of nickel.

25 Accurate control of the temperature throughout the hot rolling operation is also an important factor in the working of copper-zinc and copper-nickel-zinc alloys of the above mentioned compositions. The hot rolling temperatures of these alloys should never be allowed to fall below the "critical" temperatures, which are approximately 1350° F. and 1450° F., respectively, for the copper-zinc and the copper-nickel-zinc alloys referred to. Furthermore, the hot rolling temperature for these alloys should never exceed a predetermined maximum, which is 1550° F. for the copper-zinc alloys containing 63 to 68 per cent of copper, 1650° F. for the copper-nickel-zinc alloys containing 53.5 to 56.5 per cent of copper and 16.5 to 19.5 per cent of nickel, and 1750° F. for the copper-nickel-zinc alloys containing 70.5 to 73.5 per cent of copper and 16.5 to 19.5 per cent of nickel.

30 As an illustration of the practice of the invention the following example is given:

A copper-zinc alloy containing 66 per cent of copper is cast into a billet substantially free of impurities and containing not more than 0.1 per cent, preferably less than 0.05 per cent of lead. 5 The billet is heated to approximately 1500° F. in the furnace 1, and is then passed through the hot rolls 3-4 where its thickness is reduced in five passes from two and one-half inches to .150 inches, each pass reducing the thickness of the metal by about 40 to 45 per cent. Preferably by 10 controlling the speed of rolling the resulting sheet emerges from the hot rolls at a temperature above 1350° F., and it is then allowed to cool in air, thereby annealing the metal. The sheet is then 15 pickled and is next passed through the cold rolls 9, 10 and 11, where its thickness is reduced from .150 inches to .020 inches, each pass reducing the thickness of the metal by about 50 per cent. The metal is now placed in the annealing oven 12 and 20 annealed in the usual manner, after which it is reduced to a final gauge of say .018 inches by the cold rolls 14, which cold rolling operation imparts a definite and predetermined degree of hardness 25 to the metal, corresponding to the amount of reduction in thickness from .020 inches to .018 inches. If the metal is to be finished soft, the rolling through rolls 14 is omitted, rolls 11 being so adjusted as to reduce the sheet to the desired thickness.

30 Although the invention has been described with particular reference to certain embodiments thereof, various modifications may be made therein, and it is intended to claim such modifications as fall within the terms of the appended claims.

What is claimed is:

1. A method of forming sheets of a copper-zinc alloy containing from 63 to 68 per cent of copper, which comprises heating a billet of said 40 alloy to a temperature between 1350° F. and 1550° F. and hot rolling the billet to a sheet while maintaining the temperature thereof within in said range.

2. A method of forming sheets of a copper-zinc alloy containing from 63 to 68 per cent of copper, which comprises casting a billet of said 45 alloy containing not more than 0.1 per cent of lead, heating the billet to a temperature between 1350° F. to 1550° F., and reducing the billet to a sheet while maintaining the temperature thereof within said range.

3. A method of forming sheets of a copper-zinc alloy containing from 63 to 68 per cent of copper, which comprises casting a billet of said alloy containing not more than 0.05 per cent of lead, and 55 hot rolling the billet into a sheet while maintaining the temperature thereof above 1350° F.

4. A method of forming thin sheets of a copper-zinc alloy containing from 63 to 68 per cent of copper, which comprises hot rolling a billet of 60 said alloy into a sheet while maintaining the temperature thereof above 1350° F., and then cold rolling the sheet to substantially the desired gauge.

65 5. A method of forming sheets of a copper-nickel-zinc alloy containing from 53.5 to 73.5 per cent of copper and 16.5 to 19.5 per cent of nickel, which comprises casting a billet of said alloy containing not more than 0.1 per cent of lead, heating the billet to a temperature between 70 1450° F. to 1650° F., and reducing the heated billet to a sheet while maintaining the temperature thereof within said range.

6. A method of forming sheets of a copper- 75 nickel-zinc alloy containing from 53.5 to 56.5 per

cent of copper and 16.5 to 19.5 per cent of nickel, which comprises heating a billet of said alloy to a temperature between 1450° F. and 1650° F., and reducing the heated billet to a sheet while maintaining the temperature thereof within said range. 5

7. A method of forming sheets of a copper-nickel-zinc alloy containing from 70.5 to 73.5 per cent of copper and 16.5 to 19.5 per cent of nickel, which comprises heating a billet of said alloy to 10 a temperature between 1450° F. to 1750° F., and reducing the heated billet to a sheet while maintaining the temperature thereof within said range.

8. A method of working a copper-zinc alloy 15 containing 63 to 68 per cent copper and substantially free of impurities which comprises heating a billet of said alloy to a temperature between 1350° F. and 1550° F., hot rolling the billet to form a sheet by such reductions as to maintain 20 the temperature in said range, cooling the sheet at a rate to effect an annealing thereof, and cold rolling the sheet to the desired gauge.

9. A method of forming sheets of a copper-zinc alloy containing from 63 to 68 per cent of copper, 25 which comprises heating a billet of said alloy to a temperature between 1350° F. and 1550° F. and hot rolling the billet to a sheet by such reductions and at such a rate as to maintain the temperature thereof within said range, allowing 30 the sheet to cool to effect an annealing thereof, and cold rolling the sheet.

10. A method of forming sheets of a copper-zinc alloy containing from 63 to 68 per cent of copper, which comprises casting a billet of said 35 alloy containing not more than 0.1 per cent of lead, heating the billet to a temperature between 1350° F. to 1550° F., reducing the billet to a sheet by such reductions and at such a rate as to maintain the temperature thereof within 40 said range, allowing the sheet to cool to effect an annealing thereof, and cold rolling the sheet.

11. A method of forming sheets of a copper-zinc alloy containing from 63 to 68 per cent of copper, which comprises casting a billet of said 45 alloy containing not more than 0.05 per cent of lead, heating the billet to a hot rolling temperature, hot rolling the billet into a sheet by such reductions and at such a rate as to maintain the sheet at the hot rolling temperature, allowing 50 the sheet to cool to effect the annealing thereof, and cold rolling the sheet.

12. A method of forming sheets of a copper-zinc alloy containing from 63 to 68 per cent of copper, which comprises casting a billet of said 55 alloy containing not more than 0.05 per cent of lead, hot rolling the billet into a sheet while maintaining the temperature thereof above 1350° F., allowing the sheet to cool to provide an annealed sheet, and cold rolling the annealed sheet 60 to the desired gauge.

13. A method of forming sheets of a copper-nickel-zinc alloy containing from 53.5 to 73.5 per cent of copper and 16.5 to 19.5 per cent of nickel, which comprises casting a billet of said 65 alloy containing not more than 0.1 per cent of lead, heating the billet to a temperature between 1450° F. to 1650° F., reducing the heated billet to a sheet by such reduction and at such a rate as to maintain the temperature thereof within 70 said range, allowing the sheet to cool to provide an annealed sheet, and cold rolling the annealed sheet to the desired gauge.

14. A method of forming sheets of a copper-nickel-zinc alloy containing from 53.5 to 56.5 per 75

cent of copper and 16.5 to 19.5 per cent of nickel, which comprises heating a billet of said alloy to a temperature of 1450° F. and 1650° F., reducing the heated billet to a sheet by such reductions and at such a rate as to maintain the temperature thereof within said range, allowing the sheet to cool to effect an annealing thereof, and cold rolling the annealed sheet to the desired gauge.

15. A method of forming sheets of a copper-nickel-zinc alloy containing from 70.5 to 73.5 per

cent of copper and 16.5 to 19.5 per cent of nickel, which comprises heating a billet of said alloy to a temperature of 1450° F. to 1750° F., reducing the heated billet to a sheet by such reductions and at such a rate as to maintain the temperature within said range, allowing the sheet to cool to provide an annealed sheet, and cold rolling the annealed sheet to the desired gauge.

5  
SAMUEL McMULLAN.  
ELMORE STEELE STRANG. 10